

Nov. 7, 1939.

J. EGGERT ET AL

2,179,228

PROCESS OF COLOR PHOTOGRAPHY AND MATERIAL THEREFOR

Original Filed March 12, 1935



Inventors:  
John Eggert  
Alfred Grosshickler,  
By Attorneys Bruno Wendt,  
Potter, Pierce & Scheffler.

Patented Nov. 7, 1939

2,179,228

# UNITED STATES PATENT OFFICE

2,179,228

## PROCESS OF COLOR PHOTOGRAPHY AND MATERIAL THEREFOR

John Eggert, Leipzig-Gohlis, and Alfred Froehlich and Bruno Wendt, Dessau, Germany, assignors, by mesne assignments, to Agfa Ansco Corporation, Binghamton, N. Y., a corporation of Delaware

Application March 12, 1935, Serial No. 10,704.  
Renewed April 11, 1939. In Germany March  
16, 1934

15 Claims.

(Cl. 95—6)

Our present invention relates to color photography.

One of its objects is to provide an improved process of color photography. Another object is 5 a material for this improved process. Further objects will be seen from the detailed specification following hereafter.

For the production of colored photographic pictures by color synthesis by means of azo-dye-stuffs there have hitherto been available two 10 principal procedures. One procedure depends on the use of a diazo-component which is not stable towards light (diazotype process), whilst in the other use is made of the silver image in 15 order to produce a colored image by way of a reactive silver compound. Particularly in the latter case it is endeavoured to incorporate one or both of the dyestuff components in the light-sensitive layer as far as possible in a water insoluble, stable form resistant to the development 20 and fixing baths, and in such a manner that the transparency, natural sensitivity and artificial sensitization of the layer are not diminished.

It has been proposed, for example, to add the 25 dyestuff components to the photographic layer in the form of compounds insoluble in water, such as metal compounds, salts of organic acids or, in the case of acid components, in the form of esters, anilides or the like. These compounds are to 30 be finely dispersed, for example, by introducing into the gelatin an alcoholic solution of the compound which is insoluble in water, so that the compound is precipitated in the photographic layer. In this manner it is possible to incorporate 35 the compounds in the gelatin in such a fine state of distribution that notwithstanding the insolubility of the compound in water the gelatin dries to a transparent layer. Another procedure for adding dyestuff components to the gelatin in water insoluble form makes use of coupling components which can be fixed by mordanting. Such 40 coupling components, for example, naphthol, chromotropic acid or the like, can be fixed on the gelatin with the aid of a metal oxide and provided 45 that the component has a suitable constitution the gelatin will dry to a layer clear as glass.

The present invention is based on the discovery 50 that it is possible to incorporate in the photographic layer azo-components from aqueous solutions in such a manner that they are resistant towards the usual photographic baths by choosing those azo-dyestuff components which have substantive properties with respect to the layer. The addition of these substantive components naturally does not in any way impair the

transparency of the layer whilst the capacity of the compounds for coupling is completely preserved, since in contrast to other processes the compounds are not distributed heterogeneously in the layer but are actually dissolved in the 5 gelatin.

The procedure for carrying out the invention may consist for example, in adding to a solution 10 of gelatin or the like a solution of an azo-component or diazo-component which is substantive towards gelatin, whereupon the gelatin is thoroughly washed with water and then worked up in the usual manner. It is also possible to treat a gelatin layer or a foil of gelatin with a solution 15 of one of the aforesaid dyestuff components. In both cases the gelatin, in the language of the dyeing industry, is dyed by the dyestuff component even though in the case of a colorless component the layer does not acquire a color which 20 can be perceived by the eye.

In order to produce a colored image use may be 25 made of any of the known processes.

For instance gelatin which has been treated with both dyestuff components may be worked 30 up into a silver halide emulsion. After exposure the silver image is bleached in a bleaching bath which at the same time tans and hardens the 35 gelatin at the exposed parts of the layer. If now the layer is treated with an acidified solution of sodium nitrite, diazotization and formation of a dyestuff occur at those parts of the picture area 40 which are not hardened and are therefore accessible to the action of the nitrite solution. In this manner a red picture may be obtained by means of 2:3-hydroxynaphthoic-acid- $\alpha$ -naphthalide corresponding with the formula



and urea-bis-(para-aminobenzoyl-para-phenylene-diamine-sulfonic acid corresponding with the formula



In this method it is also possible to incorporate 50 in the gelatin only the azo-component and to use instead of the nitrite solution a diazo-solution. Thus by dyeing the gelatin with 2:3-hydroxynaphthoic-acid- $\alpha$ -naphthalide and treating the layer with tetrazotized dianisidine there is obtained a blue picture. Another procedure may 55

consist in dyeing the gelatin only with the azo-component and then either converting the silver image into an anti-diazotate image (for example according to U. S. Patent No. 1,963,197) or causing the silver halide to adsorb a diazonium compound and after washing forming the dyestuff in a coupling bath. For example, if the gelatin is dyed with di-ortho-sulfobenzylidene-4:4'-diaminodiphenylurea corresponding with the formula



a yellow picture may be obtained by means of the anti-diazotate of  $\beta$ -naphthylamine. Furthermore, there can be used instead of the 2:3-hydroxynaphthoic acid arylides similarly constituted hydroxycarboxylic acid amides, for instance, arylides of 2:3-hydroxyanthracenic acid, arylides of hydroxycarbazole carbonic acid, arylides of hydroxynaphthocarbazole carboxylic acid (a compound of this group corresponds with the formula



30 or arylides of terephthalacetic acid (a compound of this group corresponds with the formula



arylides of the hydroxycarboxylic acid of diphenylene oxide and diphenylene sulfide (compounds of this group corresponds with the formulae



and



furthermore the arylides of  $\alpha$ -naphthindole-2-phenyl-7-hydroxycarboxylic acid (a compound of this group corresponds with the formula



60 as well as pyrazolones from 2-p-aminophenylthiazoles (a compound of this group corresponds with the formula



and 2-hydroxyfluoren,  $\beta$ -hydroxyanthracen, hydroxychrysene and others. A like picture is obtained if the silver halide is caused to adsorb para-nitro-benzenediazonium-chloride and coupling is then brought about.

Yet a further procedure in accordance with the invention consists in dyeing the gelatin with both dyestuff components and then converting the silver image into an insoluble nitrite compound.

If now diazotization is brought about in any suitable manner the dyestuff is formed at the places in the layer corresponding with the image. In this manner a red picture may be produced, for example, from the urea from para-dimethylaminobenzoyl-para-aminobenzoyl-2-amino-5-naphthol-7-sulfonic acid corresponding with the formula



and the urea-bis-(para-aminobenzoyl-para-phenylenediamine-sulfonic acid).

The foregoing examples illustrate only some of the possible procedures and the invention is realized in any case in which, for the production of an azo-dyestuff image, one or both of the components or the diazo-component in its undiazotized form has a substantive character with respect to the binding agent or to the support for the layer.

Compounds which have proved to be especially suitable for use in the invention are, for example, the aminobenzoyl-aminobenzoyl compounds of aminonaphthol sulfonic and carboxylic acids (a compound of this group corresponds with the formula



45 of naphthylamine sulfonic and carboxylic acids (a compound of this group corresponds with the formula



55 of cresotinic acid and of diaminocarbazole disulfonic acid (a compound of this group corresponds with the formula



75 as well as the ureas from the aminobenzoyl compounds of the aforesaid coupling components (a

compound of this group corresponds with the formula



Of particular interest are further the benzoyl-, benzyl- and benzylidene-compounds of diaminodiphenyl ureas, of diaminodiphenyl-thioureas, of diaminostilbenes, of benzidines and similar compounds (compounds of these groups correspond with the formulae



including compounds containing any substituents in any positions.

The invention is of particular importance in its application to the production of photographs in natural colors. If there are cast in superimposed relationship emulsions of which each is sensitized for one of the primary colors and is dyed with appropriate dyestuff components, the color synthesis can be conducted in the layers in the manner already described. It is possible in this manner to obtain polychrome pictures without the use of transfer processes and without having to dye the layer on one side only. However, it is not necessary that all the three-color pictures shall be produced by the process of the invention. On the contrary the invention can easily be combined with other processes for producing colored photographic images. For example, in the case of a three-color film two color images may be produced on one side of the support by the process of the invention, whereas the remaining color image may be produced, for example, on the other side of the support by toning or on the same side by an imbibition process.

55 The invention comprises a photographic material consisting of a support coated on one or both sides with one or more layers of silver halide gelatin emulsion which is or are dyed with an azo-dyestuff component or components substantive with respect to the layer.

60 The following examples serve to illustrate the invention:

*Example 1*

A film coated with a layer of gelatin is bathed in the following solution:

1000 cc. of water

5 grams of 2,3-hydroxynaphthoic acid dianisidine dissolved in

70 50 cc. of methanol and

10 cc. of a caustic soda solution of 20% strength

whereupon the material is washed with water for about  $\frac{1}{2}$  hour. Then the sheet is bathed in a solution of p-diphenylamindiazonium sulfate and is dried. After exposure under an original and

treatment with an aqueous solution of ammonia or gaseous ammonia a blue picture is produced at the places which were not illuminated.

*Example 2*

There is produced a solution of

10 grams of p-dimethylamidobenzoyl-p-amido-benzoyl-(2-amino-5-naphthol-7-sulfonic acid) in

1000 cc. of water, with the addition of

10 cc. of a caustic soda solution of 20% strength.

In this solution a silver bromide emulsion layer is bathed for 10 minutes and washed with water for about 1 hour. An original is printed on this layer, and the layer developed, fixed and the silver image bleached by means of copper chloride. The bleached-out silver image is converted into  $\beta$ -naphthylamine-antidiazotate-silver by means of an alkaline solution of  $\beta$ -naphthylamine-antidiazotate-sodium and thoroughly washed. When this picture is immersed into a solution of 1 gram of citric acid and 1 gram of potassium bromide, a red azo-dye picture is produced. The silver bromide is removed by fixing.

*Example 3*

There is made a solution of

20 grams of 2,3-hydroxynaphthoic-acid- $\beta$ -naphthalide in

1000 cc. of water and

10 cc. of a solution of caustic soda of 20% strength.

The solution is filtered and mixed with a solution of 10 grams of urea-bis-(p-amidobenzoyl-p-phenylenediamine sulfonic acid) in a quantity of water as small as possible and a small amount of caustic soda solution; a silver bromide emulsion layer is bathed therein for about 10 minutes, washed with water for about 1 hour and dried. When printing on this layer and converting the silver image in known manner into an insoluble nitrite compound, a red dye picture is produced by starting diazotization by bathing the layer in dilute acetic acid.

*Example 4*

100 cc. of silver bromide emulsion are mixed with a solution of

0.5 gram of 2,3-hydroxynaphthoic-acid- $\alpha$ -naphthalide in

10 cc. of a caustic soda solution of 5% strength.

Furthermore there is added a solution of

0.3 gram of urea-bis-(p-amidobenzoyl-p-phenylenediamine-sulfonic acid) in

20 cc. of caustic soda solution of 5 percent strength.

The caustic soda is neutralized by means of acetic acid the emulsion solidified and washed with water. The emulsion is cast and the silver image produced in the emulsion layer by printing, developing and fixing is bleached with a bleaching bath having the property to tan the gelatin at the places of the picture. If the picture is treated with a solution of 5 grams of sodium nitrite in 200 cc. of acetic acid of 1% strength, a dye picture is produced from the two components at the non-hardened places.

*Example 5*

(a) 1 kilo of silver bromide emulsion is mixed with 5 grams of 2,3-hydroxynaphthoic-acid-dianisidine dissolved in

25 cc. of methanol

5 cc. of a caustic soda solution of 20% strength and neutralized with 15 cc. of acetic acid of 10% strength. This emulsion is sensitized for green.

- (b) 1 kilo of silver bromide emulsion is mixed with 5 grams of urea from 1(3'-amidophenyl)-3-methyl-5-pyrazolone by conversion with phosgene

5 25 cc. of methanol and 5 cc. of caustic soda solution of 20% strength are neutralized with 15 cc. of acetic acid.

The two emulsions (a) and (b) are each hardened with 4 cc. of formaline and then the emulsion (a) is cast on one side of a film provided on both sides with a sub-layer. Then there is applied to the emulsion layer an intermediate layer of hardened gelatin of  $2\mu$  thickness containing a yellow filter dye which is destroyed in the developer. The emulsion (b) is now cast on the intermediate layer. On the other side of the support there is cast a layer of a red filter dye which is decolorized in the developer, and a panchromatic silver bromide emulsion is cast on the filter layer. Now a partial color picture is produced in each of the layers, but after development and fixing only that side of the film is bleached to which the two emulsion layers (a) and (b) have been applied. The bleached-out silver pictures are converted into  $\beta$ -naphthylamine-antidiazotate-silver pictures in the manner indicated in Example 1. If these pictures are treated with the solution of coupling component indicated in Example 1, a yellow dye picture is produced in the layer (a) and a red dye picture is produced in the layer (b). The silver picture on the opposite side of the support is converted into a blue picture by dye-toning, for instance, an iron blue picture.

In the single figure of the accompanying drawing there is shown a photographic material accompanying to this invention. The support *a* is provided with a photographic layer dyed with a compound having substantive properties with respect thereto.

What we claim is:

  1. A process of producing color photographs, which comprises incorporating in a silver halide gelatin emulsion a coupling component of an azo dye, said coupling component having a chemical constitution which imparts to said component substantive properties towards the gelatin, forming a light-sensitive layer from said emulsion, exposing said layer to light controlled by an object to be reproduced, developing the latent silver image, and causing said coupling component to react with a diazo compound, thereby producing an azo-dyestuff picture in situ with the silver picture.
  2. A process of producing color photographs, which comprises treating a silver halide emulsion layer with a solution of a coupling component of an azo dye, said coupling component having a constitution which imparts thereto substantive properties towards the gelatin, forming a light-sensitive layer from said emulsion, exposing said layer to light controlled by an object to be reproduced, developing the latent silver image, and causing said coupling component to react with a diazo compound, thereby producing an azo-dyestuff picture in situ with the silver picture.
  3. A process of producing color photographs, which comprises treating a gelatin solution containing silver halide with a solution of a coupling component having a chemical constitution which imparts thereto substantive properties with respect to the gelatin, forming a light-sensitive layer from said emulsion, exposing said layer to light controlled by an object to be reproduced, de-

veloping the latent silver image, and causing said coupling component to react with a diazo compound, thereby producing an azo-dyestuff picture in situ with the silver picture.

4. A light-sensitive photographic element comprising a support and at least one silver halide emulsion layer capable of being converted into a colored picture by exposure to light, development and treatment with a diazo compound, said silver halide emulsion layer containing a coupling component of an azo dye, said coupling component having a chemical constitution which imparts thereto substantive properties with respect to the gelatin. 5 10

5. A process of producing color photographs, which comprises incorporating in a silver halide gelatin emulsion a diazo compound and a coupling component of an azo dye, said diazo compound and said coupling component having a chemical constitution which imparts thereto substantive properties towards gelatin, forming a light-sensitive layer from said emulsion, exposing said layer to light controlled by an object to be reproduced, developing and fixing said layer, bleaching said layer in a bath which has at the same time a tanning and hardening action on the gelatin of the exposed parts of the layer, and treating said layer with an acidified solution of sodium nitrite. 15 20 25

6. A light sensitive material for color photography comprising a support and a silver halide gelatine emulsion thereon, containing an organic colorless dyestuff component capable of reacting with a further component to produce a dye-stuff image, said first component having a chemical constitution which imparts thereto substantive properties with respect to the gelatine 35

7. A light sensitive material for color photography comprising a support and a silver halide gelatine emulsion thereon, containing an organic colorless dyestuff component capable of reacting with a further component to produce a dye-stuff image, said first component containing an organic group which imparts to said component substantive character with respect to the gelatine. 40

8. A light sensitive element as defined in claim 6 wherein said first component contains at least 3 organic rings. 45

9. A light sensitive material for color photography comprising a support, a plurality of silver halide gelatine emulsions carried by said support, each emulsion containing an organic colorless dyestuff component capable of reacting with a further component to produce a dyestuff image different in color from that produced in the other layers, said first component having a chemical constitution which imparts thereto substantive properties with respect to the gelatine. 50 55

10. A light-sensitive element as defined in claim 6, wherein said first component contains at least 3 organic rings, at least 2 of said rings being selected from the class of fused rings and rings connected together by a linkage selected from the class consisting of a direct nuclear carbon to nuclear carbon linkage, a  $-\text{CH}=\text{N}-$  linkage, a  $-\text{NHCO}-$  linkage, a  $-\text{NH}-\text{CO}-\text{HN}-$  linkage, a  $-\text{NH}-\text{CS}-\text{NH}-$  linkage, a  $-\text{CH}_2-\text{NH}-$  linkage and a  $-\text{CH}=\text{CH}-$  linkage. 60 85

11. A light-sensitive element as defined in claim 6, wherein said first component contains at least 3 organic rings, at least 2 of said rings being fused together. 70

12. A light sensitive element as defined in claim 6, wherein said first component contains at 75

least 3 organic rings, at least one ring being heterocyclic.

13. A light-sensitive material for color photography comprising a support and a silver halide gelatin emulsion thereon containing an hydroxynaphthoic acid arylide containing an organic group which imparts to said compound substantive character with respect to the gelatin.

14. A light-sensitive material for color photography comprising a support and a silver halide gelatin emulsion thereon containing a pyrazolone containing an organic group which imparts to said compound substantive character with respect to the gelatin.

15. A light-sensitive material for color photography comprising a support and a silver halide gelatin emulsion thereon containing an organic

colorless dyestuff component capable of reacting with a further component to produce a dyestuff image, said first component containing at least 3 organic rings, at least 2 of said rings being selected from the class of fused rings and rings connected together by a linkage selected from the group consisting of a direct nuclear carbon to nuclear carbon linkage, a  $-\text{CH}=\text{N}-$  linkage, a  $-\text{NHCO}-$  linkage, a  $-\text{NH}-\text{CO}-\text{NH}-$  linkage, a  $-\text{NH}-\text{CS}-\text{NH}-$  linkage, a  $-\text{CH}_2-\text{NH}-$  linkage and a  $-\text{CH}=\text{CH}-$  linkage, said components although being soluble in aqueous solutions being fast to diffusion in the gelatin.

JOHN EGGERT. 15  
ALFRED FROEHLICH.  
BRUNO WENDT.